

Jan. 14, 1936.

R. R. RIDGWAY ET AL

2,027,787

WIRE DRAWING DIE

Filed Nov. 13, 1933



WITNESSES

Franklin E. Johnson  
W. R. Greenwood

By Clayton R. Jenkins  
Attorney

Inventors

RAYMOND R. RIDGWAY  
BRUCE L. BAILEY

## UNITED STATES PATENT OFFICE

2,027,787

## WIRE DRAWING DIE

Raymond R. Ridgway and Bruce L. Bailey, Niagara Falls, N. Y., assignors to Norton Company, Worcester, Mass., a corporation of Massachusetts

Application November 13, 1933, Serial No. 697,744

11 Claims. (Cl. 205—29)

This invention relates to dies, and more particularly to metal shaping dies and to a method of making the same.

The value of a wire drawing die is largely dependent on the length of wire which can be drawn to size through a given die after its opening has been carefully shaped to produce a given wire size. The limits and variations permitted in drawn wires varies over a large range. In some cases wire must be held to very close limits in the drawing. A satisfactory die, therefore, must be made of a hard material which will resist the abrading action resulting from the travel of hundreds of thousands of feet of wire through the die opening. Wire varies greatly in the nature of its abrading action on the die and in the mechanical forces imposed by the reduction process as the wire is drawn through the die opening. In the present state of the art there are four materials generally used for wire drawing dies. These are crystalline diamonds, cemented tungsten carbides, sapphires, and chilled iron alloys.

The use of diamonds for wire drawing is distinctly limited by the fact that this material is expensive as a raw material and can be had only in relatively small nib sizes. Another defect of the diamond is related to the fact that it is a product of nature which varies widely in its physical and chemical composition giving wide variations in its resistance to the strains involved and in its wearing qualities. The same general defects occur in the case of sapphires. The chilled iron alloys which have formerly been used in large quantities for the drawing of various types of wire are relatively inexpensive to manufacture but they are so easily worn by the wire drawing operation that only a relatively short length of wire can be drawn before a new die must be provided.

The cemented carbide alloys are substituted in many operations for the chilled iron alloys because their life is so much greater due to their increased wear resistance that it is economical to use the more expensive cemented carbide material. The cemented carbide alloys have a wear resistance greater than the chilled iron alloys coupled with a certain degree of strength to resist the strains produced in drawing which tend to split the die. In practice cemented carbide alloys have certain definite defects. They are much more expensive than the dies formerly used for the purpose and while they have a greater wear resistance than the chilled iron alloys, they are made of materials of two definite degrees of hardness so that they cannot be finished to a high polish and, therefore, the reduction area and bearing surfaces offer friction to the drawing of wire and place a certain amount of scratches on the drawn product. The cemented

carbide die, therefore, cannot fully replace crystalline material such as diamond where the bearing surface in the die can be highly polished. The hardness of the cemented carbide alloys is not equal to that of the diamond and, therefore, the wear resistance of the finished die is not the equivalent of a diamond die. 5

It is the primary object of this invention to produce a die which will be free from the unfavorable characteristics of the diamond and yet 10 will have some of its desirable properties, namely its crystalline nature and its high degree of wear resistance. Further objects will be apparent from the following description.

In accordance with this invention we propose 15 to make such dies of boron carbide and thus to overcome various problems heretofore met in the industry. The boron carbide of commerce has heretofore consisted of a black powder of variable and uncertain composition. It has been 20 contaminated with a high degree of free graphite and other metallic impurities such as boron, iron, aluminum silicon, and the like. Such a material is of no use for the manufacture of wire drawing dies and cannot be manufactured into a body 25 suitable for a wire drawing nib.

In the course of our experimentation, we have discovered that the unusual properties of boron carbide of the formula  $B_4C$ , or as made in accordance with the method described in the patent to Ridgway No. 1,897,214 of February 14, 1933, make this material particularly well adapted for use as a metal shaping or drawing die, such as dies for drawing wire, tubes, etc., or for extrusion operations and other purposes. This 30 boron carbide is characterized by a hardness approaching that of the diamond. It is wear-resistant or durable and is particularly suited for use under the action of abrasion during a drawing operation. It is only slightly below the diamond in the scale of hardness, besides being appreciably harder than the standard abrasive materials, such as tungsten carbide, crystalline alumina and silicon carbide. The boron carbide, as described, is further characterized by having a 35 glassy conchoidal fracture and appearing as a dense, homogeneous mass having a single phase of crystalline boron carbide without intergranular weakness. The material is particularly characterized by its being devoid of parting planes of 40 graphite and uncombined carbon, and it is undiluted by any foreign and undesired impurities, such as borides and carbides of iron, aluminum, silicon and other metals. It has a very high melting point of about  $2300^\circ +$  or  $- 100^\circ C.$  and 45 probably melts at about  $2275^\circ C.$ , as measured by optical methods. The boron carbide is very stable and is not decomposed by the furnace heat, and in particular it does not vaporize in the manner in which boron metal does, but it melts 50

to a liquid phase and crystallizes therefrom so that it is capable of being formed into a molded shape. Hence, it is, therefore, particularly desirable for use as a material for a wire drawing die, due to its superior abrasion resistance, and when suitably mounted and supported it is strong enough to withstand the large stresses which tend to split the die in use.

In accordance with our invention, we so make the die nib or body that its effective portion comprises boron carbide, as above described, and is so constituted as to be adapted for a metal shaping operation. We propose to shape the boron carbide, as made in accordance with the Ridgway patent, by a suitable procedure, in accordance with which the effective surface of the die is so made as to contain this extremely hard material in sufficient proportion to satisfy the desired ends. It is necessary that cementing matrices or impurities be present only in relatively small amounts. We prefer to make the die in accordance with the disclosure in our copending application Serial No. 694,502 filed October 26, 1933, whereby we mold the  $B_4C$  material into a unitary body having a substantially continuous one-phase crystalline structure. The material may be molded into a desired shape for use as a die, either with or without the die opening under high temperature furnacing conditions which cause the boron carbide to be melted or softened and shaped by a mold and then crystallized into a one-phase crystalline body of high density, and preferably of from 2.3 to 2.55. The process is preferably so carried on that the body is not contaminated in particular with substantial amounts of dissolved graphite and does not contain parting planes of graphite within its mass and which, therefore, has great strength, density and rigidity as well as hardness.

This method is preferably accomplished by heating boron carbide powder of a required degree of purity and grain size to a temperature at which it will melt or soften and be capable of being molded, after which the material may be shaped under pressure in a mold of suitable refractory material, while conditions are maintained which prevent the  $B_4C$  material from reacting chemically with or physically dissolving foreign substances capable of detrimentally affecting the properties of the die. Since boron carbide dissolves carbon readily, the manufacture of the die is arranged so that the material is heated to a softened condition and caused to be shaped while it is too viscous, or insufficiently heated, to dissolve or react with the graphite mold parts to any detrimental extent. If the material is fully melted so as to become completely fluid, it is desirable then that it be rapidly cooled, after it has assumed its final shape, to a temperature at which it is stable. In this way, the material is not permitted to remain in contact with graphite while in the molten state, or only for the minimum of time required for it to become shaped by the mold under the conditions of the molding or casting operation.

In the forming operation, it is desirable that the process be carried on in the presence of an inert atmosphere or in the absence of oxygen or other substances which cause oxidation or decomposition of the boron carbide. It is also essential that the material be prevented from absorbing more carbon than is necessary to satisfy the ratio of  $B_4C$ . Our experiments have also indicated that liquefaction or softening of the boron carbide powder may be brought about at

a temperature appreciably below its melting point when it is subjected to a high pressure. Under such conditions of temperature and pressure, liquefaction of the compound may be attained without the solution of additional carbon over what is necessary to produce the form of boron carbide as set forth in the Ridgway patent. It has also been found, by experimental tests, that the material crystallizes again when the pressure is released, even though the temperature is held constant.

The following examples from test records show a comparison between typical analyses of the composition of the boron carbide powder before molding into the form of a metal drawing die and the composition of the formed pieces resulting from the high temperature molding process.

|                                                         | Percent by weight |      |    |    |    |    |       | 20 |
|---------------------------------------------------------|-------------------|------|----|----|----|----|-------|----|
|                                                         | B                 | C    | Si | Fe | Al | Ca | MgO   |    |
| Composition of boron carbide powder before molding..... | 76.5              | 20.6 | .8 | .4 | .3 | .1 | Trace | 25 |
| Composition of pieces molded from above powder          |                   |      |    |    |    |    |       | 30 |

  

| Composition of pieces molded from above powder | Percent by weight |      |    |       |       |      |      | 30 |
|------------------------------------------------|-------------------|------|----|-------|-------|------|------|----|
|                                                | B                 | C    | Si | Fe    | Al    | Ca   | MgO  |    |
| Sample No. 1.....                              | 77.3              | 22.4 | .3 | .1    | .2    | None | None | 35 |
| Sample No. 2.....                              | 77.8              | 21.0 | .7 | .3    | .2    | "    | "    |    |
| Sample No. 3.....                              | 78.5              | 21.1 | .3 | Trace | Trace | "    | "    |    |

In practice, it has been found advantageous to maintain in the boron carbide powder a small amount of free uncombined boron in excess over that required to make the carbide set forth in the aforementioned Ridgway patent. It may be assumed that this excess of uncombined boron metal will act to neutralize or react with the carbon vapors resulting from the carbon mold and the related parts.

In the examples above noted, it will be seen that the high temperature molding operation used in making the molded article results in the composition taking up additional carbon, with the consequent decrease of the free boron content, as compared to the ideal composition desired, and the further reduction of the small amounts of impurities, by volatilization, to insignificant quantities. In the above table, it will also be observed that the analysis of Sample No. 3 approach closely to the ideal composition.

In forming a die in accordance with this invention, the boron carbide in a finely divided condition or powdered form is subjected to pressure while it is heated to a point at which it becomes molten or sufficiently soft to be molded, the pressure being sufficiently high to consolidate the particles into a structure of the required density and other characteristics. To attain the maximum apparent density, a boron carbide powder having a particle size not greater than will be retained on a screen having 200 meshes to the linear inch is preferably used. If coarse grains are used, with the resulting large intergranular spaces, a much larger applied pressure is required to produce the maximum density than when fine sizes are used. A fixed sizing of the grains may also be used so that a definite volume-weight relationship exists in the material to be fused into a dense mass. If such a powder of pure boron carbide is

employed, the apparent density may be raised to a value substantially equal to or within 2% of the real density of boron carbide, which is about 2.52. Also, if necessary, the carbide grains 5 may be subjected to suitable chemical treatment to remove any chemically reactive constituents from the finely divided powder in order that a substantially chemically pure boron carbide may be obtained.

10 A non-reactive refractory material should be utilized for the mold or container for the molten carbide, and we find that ordinary commercial graphite having a strong non-porous form and which has been processed to give a maximum 15 density, such as is used as an electric furnace electrode, can be used as a practical material for the mold. This graphite is well known in the electro-metallurgical art and consists essentially of pure carbon with only negligible amounts of ash constituents. Owing to the availability and cheapness of graphite, we prefer to use a graphite of 20 the purest and highest quality for this mold.

The molding apparatus is preferably equipped with a movable graphite plunger fitted into the 25 mold so that by applying pressure to the plunger, it is possible to follow the conversion of the solid carbide grains to the molten phase as the material is raised to the specified temperature, so that when fusion takes place the movement of 30 the plunger will indicate the total fusion of the grains within the container. As soon as the indication is given that the material has melted, the assembly of mold and its molten contents is immediately cooled below the melting point of 35 the boron carbide. Due to the ease with which molten boron carbide dissolves graphite, it is necessary that the material be cooled rapidly soon after it has become molten or sufficiently fused to become shaped by the graphite container. In 40 this way, the molten material is permitted to remain in contact with the graphite only for the minimum of time required for the molding operation.

In the manufacture of a molded boron carbide die, the exact conditions will be determined by the nature of the material used and the size and density of the finished product. In the manufacture of a wire drawing die which is of comparatively small dimensions but is required to be of the maximum obtainable density and to be accurately dimensioned, it is preferable to make the article in accordance with the following procedure. Boron carbide of a high degree of purity and of the required composition of boron and carbon, preferably that type of material which is obtained in accordance with the process set forth in the Ridgway Patent No. 1,897,214 and treated with acid as above described, is crushed to a suitable size, and preferably one which is finer than will be retained by a screen of 200 meshes to the linear inch. The powdered material will have a real density of approximately 2.52, and the size of the particles will be so selected and distributed as to give the maximum apparent density to avoid large plunger movements. A definite weighed amount of this carefully selected material, as predetermined by suitable calculations, is placed in the graphite mold and heated rapidly under pressure until 50 coalescence takes place. The material may be preliminarily pressed to shape in the mold or prior to its being placed in the mold so that it will have an apparent density of about 2.0, thus lessening the plunger movement during the pressure casting operation.

It has not definitely been proved, but it may be conveniently assumed that the pressure applied to the plunger may also serve to lower the fusion point of the boron carbide grains to a point where the rate of solution of carbon from the containing walls is greatly reduced, thereby making possible the production of the fused article without the inclusion of excess graphite. The temperature range within which the product has been found to have useful properties has been 10 from 2000° C. up to 2500° C. However, by applying sufficient pressure to insure the required density of product, and by carefully limiting the temperature so as to reduce it below the melting point as soon as the material has been sufficiently 15 heated to shape it to the mold, a boron carbide article may be made which has not dissolved material amounts of carbon from the graphite mold. If desired, the plunger movement during the casting operation may be so controlled that a definite 20 amount or weight of grains which has been calculated to occupy a desired volume percentage of the final product will be caused to occupy that volume in the shaped body, so that the porosity will likewise constitute a desired volume. 25

The amount of pressure to be applied to the materials in the mold will be determined in accordance with the size and desired density of the die to be made. For example, in making dies, the pressure limits may be maintained within a range 30 of from 1000 to 5000 lbs. per sq. in. to produce articles of the highest quality. Use of greater pressures may result in failure due to destruction of the mold parts, whereas the employment of lower pressures will not result in the production 35 of a product of sufficiently high density.

In the case of the manufacture of nibs of very small dimensions such as are ordinarily used for the drawing of small wires, we have found that it is necessary to use the higher range of pressures 40 in order to produce a satisfactory piece. This is related to the mold friction which serves to neutralize the pressure applied to the plungers. Therefore, in the manufacture of dies of highest quality, the highest pressure which is consistent with the strength of the plunger should be applied due to the small total pressure which is called for by a small nib. The ordinary frictional losses are abnormally high in proportion to the total applied force. We have also observed in 50 practice that there is a certain tendency for the powder in the mold to pack and resist the pressure of the plunger due to friction along the side of the mold. In such cases, accuracy and success of the molding operation depends upon the 55 use of sufficiently high pressure to overcome this effect and also requires a smooth and highly polished mold surface. In practice, we have found that the point of highest density is that part of the finished article which is nearest to the 60 plunger.

For a die nib of approximately 0.600" outside diameter and approximately 0.300" thickness with conical depressions, one on each face but without the molded hole, a pressure of 3300 lbs. 65 per sq. inch has been found satisfactory and will form a completed article with a density of from 2.4 to 2.55, when the maximum temperature reached in the formation of this piece was approximately 2250° C. In practice, it may be desirable to have the mold parts constructed so as to produce a greater density at the bearing length of the die opening which is advantageous as wear is greatest at that end, due to the pull of the wire passing through the die. 70

However, one may so control the length of the heat softening and compacting period as to keep the boron carbide from contacting with the graphite mold any longer than necessary while it is in a molten condition; and, if desired, the pressure casting operation may be stopped at a point short of that at which the material has become fully molten. The degree of pressure and temperature applied, as well as the grit size used will determine the density of the article. The pressure limits will, of course, be governed largely by the strength of the mold and the furnace materials.

It will be evident to any metallurgist that various methods are available for the refining of the grain in the products produced by the molding operation. Rates of cooling, variations of temperature, pressure, length of heating period, and original grain size of the powder all influence the structure of the resultant formed article, and their control are all within the skill of one familiar with this art.

The body thus formed has a purity in excess of 99% of B<sub>4</sub>C, and it is believed to be made up of a substantially continuous crystalline phase of boron carbide, which is substantially free from any cementing material of a low degree of hardness. The body has a conchoidal crystalline fracture and freedom from any material amount of graphite and other undesired impurities, and it appears to be similar to the boron carbide material as originally made in the electric furnace in accordance with the Ridgway patent. If a density of 2.3 or greater has been attained, the body is of a metal-like appearance capable of taking a high polish, and its modulus of rupture in compression is in excess of 100,000 lbs. per sq. in.

Referring to the drawing which illustrates one embodiment of the invention, we have there illustrated in an enlarged sectional view a molded wire drawing die nib composed of boron carbide of the formula B<sub>4</sub>C mounted in a metal backing or reinforcing holder for a wire drawing operation. This die construction is shown as comprising a wire drawing body 10, which is composed of dense, homogeneous boron carbide made in the manner above described, and having a central aperture or opening 11 of the proper design and shape suitable for wire drawing purposes and which will promote good lubrication and wire reduction during the drawing process. The die opening 11 may be formed in the boron carbide body during the pressure molding operation, or it may be drilled by suitable means after a solid body has been cast. In the latter case, either a depression may be formed in each face of the body during the casting operation and boron carbide crystals from a previous operation, or preferably diamond powder or dust may be employed with rotary iron drills in accordance with the standard practice of drilling diamond dies to form a hole between the depressions. In the pressure casting method of forming an opening, a core of suitable size may be employed in the mold, and in certain cases a hole of smaller dimensions than ultimately required may be formed during the pressure molding operation and the hole thereafter enlarged and finished by means of a suitable diamond drilling operation to the desired wire diameter.

As a result of the boron carbide die material being a crystalline material of a high degree of hardness, it is somewhat brittle in character. This necessitates a careful mounting of the nibs

in a suitable backing or a protective casing to take up the strains induced in the material by the drawing operation. The conical reduction area of the die acting on the wire during the drawing operation results in a component of force which tends to split the die. Therefore, great care must be taken in mounting the boron carbide nib in the casing to insure that the brittle die material does not bear all of the force which tends to split the die in the drawing operation. It is necessary also that the force exerted on the die nib be equally applied throughout its entire circumference so that no distortion may be produced in the hard brittle material by the forces resulting from wire drawing.

It will be apparent to those skilled in the art of mounting nibs that care must be taken to insure that the backing material is thus equally and smoothly applied to the carbide and that it has such characteristics under heat and pressure that it will continuously act to support the hard wear resisting material in all types of severe operation. To this end it is necessary to provide a backing material of the proper coefficient of expansion and tensile strength to protect the die against abusive treatment. It is recognized among die manufacturers that various wire drawing machines and types of wire drawing require suitable adaptation of reduction area angles, bearing surfaces, and back openings. The adaptation of our material to any commercial operation will be evident to one skilled in the art of die making if its properties of great hardness and brittleness are properly known.

Various methods of mounting the die nibs may be employed. For example, the die nib 10 may be mounted in a casing 12 in such a manner that it will be reinforced against the high disruptive pressure set up when drawing wire of a maximum size for the die dimensions. For this purpose, the casing 12 will be shaped to dimensions slightly larger than those of the boron carbide nib and it will be provided with a central opening 13 which is directly in line with but larger than the die opening 11 and towards and through which the wire is drawn. The die nib 10 may be brazed or cemented or otherwise secured therein. Also, since boron carbide is capable of taking a high polish or of being made to extremely accurate dimensions, it may be feasible to embed the boron carbide directly in a backing which has been accurately shaped to fit the same. In that case, the backing or reinforcing casing may be made to correct dimensions and then be heated and shrunk onto the nib. If desired, one may also employ a procedure in which the boron carbide die may be first made as smooth as possible, as by a suitable polishing operation, and then electroplated with a suitable metal, such as a heavy coating 15 of copper, after which it will be mounted in a steel holder in a hydrogen atmosphere. The holder will be heated to a sufficiently high temperature to expand it for mounting on the die, after which it may be then cooled and shrunk in place, the copper serving as a jointing material which insures perfect union between the parts. Other methods of mounting the boron carbide die are feasible, such as by copper brazing or by the use of solder sweated in a holder of nickel alloy.

It will be apparent that, in accordance with this invention, we have provided a die construction which has a long life due to the great hardness and homogeneity of the material. Moreover, the high density and consequent glass-like

smoothness throughout the bearing length of the die opening prevents undue abrasion and results in less friction in the die opening and consequently less wear and continued high production.

5 While this invention is directed to the adaptation of a pure crystalline material boron carbide such as is described in the U. S. Patent 1,897,214, formed in accordance with the copending application serial #694,502, it is within the spirit of this invention that the crystalline material may be altered by slight variations in the boron and carbon content of the product or by the addition of toughening materials in order to resist certain 10 specially abusive conditions. It must be recognized that such small additions do not change the essential nature of the die material but may be used to alter its crystallinity. This is distinct from processes where large amounts of a relatively soft cementing metal are incorporated with the hard carbide such as is well known in the cemented carbide art. It is well known to metallurgists that the crystalline properties of metals may be altered with minute additions of various 15 agents to control the crystallinity. In the metallurgy of tungsten, various agents are known which when added in amounts of 1% will modify the crystalline nature of the metal which is formed in a semi-plastic condition. It should be pointed 20 out that the product forming the die covered by this invention is essentially a single crystalline individual formed in a semi-plastic or molten condition and self-bonded, but such alterations and additions of other materials to modify the 25 crystallinity or produce various slightly altered characteristics in the die material are well within the scope of this invention, which comprises a crystalline boron carbide grown from the molten or plastic stage under pressure and consisting of upwards of 90% of boron carbide in a crystalline 30 form without cementing materials.

35 The expression "continuous crystalline phase" as found in the claims is not intended to limit this case to any particular theory of formation of the body, nor as to the physical condition of the product. It is immaterial in so far as this invention is concerned whether the individual grains have melted completely during the pressure molding operation and then have crystallized into a single 40 homogeneous body, or whether the individual grains have not been wholly melted but have been merely softened and molded together into an integral body, or have recrystallized without melting. The expression is, however, intended to 45 cover a body which is substantially devoid of parting planes of graphite and of any large amount of other impurities which can seriously interfere with the homogeneity and integrity of the body, and with its functions for the purposes 50 herein described. The body, as thus formed, is made up substantially wholly of boron carbide, depending upon the degree of purity of the materials initially employed.

55 Having thus described the invention, what we claim as new and desire to secure by Letters Patent is:

1. A die shaped as a perforated nib of required dimensions having a wire drawing surface, the effective portion of which comprises boron carbide of the formula  $B_4C$ .

70 2. A die shaped as a perforated nib of required dimensions, the effective portion of which comprises boron carbide of the formula  $B_4C$  having a substantially continuous crystalline phase and be-

ing substantially devoid of graphite and structure weakening impurities.

3. A die shaped as a perforated nib of required dimensions, the effective portion of which comprises boron carbide grains of high purity molded under heat and pressure into a body having a substantially continuous crystalline phase of boron carbide having a composition conforming substantially to the formula  $B_4C$ .

4. A die for wire drawing comprising a molded body having a substantially continuous single phase of boron carbide conforming substantially to the formula  $B_4C$  which is substantially free from parting planes of graphite and structure weakening impurities.

5. A die for wire drawing comprising a perforated body of required shape and dimensions having a wire engaging surface consisting of boron carbide granules of the formula  $B_4C$  compacted into a dense, coherent mass in which the structure of said body is made up of a single, hard constituent having a substantially continuous crystalline phase which is devoid of graphite and other impurities and being substantially free from cementing materials of a low degree of hardness.

6. A wire drawing die comprising a perforated body formed of granules of boron carbide of the formula  $B_4C$  which individually have a substantially continuous crystalline phase and are devoid of graphite and detrimental impurities and which have been molded under heat and pressure while in a softened condition to form a coherent body presenting a substantially homogeneous wire drawing surface of uniform hardness and having a density above 2.4.

7. A wire drawing die of required shape and dimensions, the effective portion of which is of a substantially continuous phase of boron carbide having a composition conforming substantially to the formula  $B_4C$  which when molded to the required dimensions and shape is substantially free from parting planes of graphite and structure weakening impurities, said article having a density between 2.4 and 2.55 and a modulus of rupture in compression in excess of 100,000 lbs. per sq. in. and being capable of taking a high polish.

8. A die for wire drawing comprising an inner perforated drawing nib of boron carbide of the formula  $B_4C$  having a substantially continuous crystalline phase which is shaped and adapted for drawing wire and a metal supporting member which makes a rigid contact with the nib and reinforces it against the pressure of a wire drawing operation.

9. A molded wire drawing die composed of boron carbide of the formula  $B_4C$  of a substantially single continuous crystalline phase, said die having a metal coating upon its outer exposed surface.

10. A molded wire drawing die composed of boron carbide of the formula  $B_4C$  of a substantially single continuous crystalline phase, said die having an electroplating of copper upon its outer exposed surface.

11. A wire drawing die comprising a molded body having a substantially continuous single phase of boron carbide of the formula  $B_4C$  and formed with a shaped aperture presenting an extremely smooth, polished, wire drawing surface, a metal coating on the molded body and a metal supporting holder integrally united thereto.

RAYMOND R. RIDGWAY.  
BRUCE L. BAILEY.